

Dec. 27, 1949

2,492,269

R. T. COMER, JR.  
FLUID COOLED MEMBER FOR BLAST  
FURNACES AND THE LIKE  
Filed Aug. 5, 1948

FIG. 2.



FIG. 1.



*Inventor:*

*ROBERT T. COMER, JR.*  
*by: Donald G. Dalton*  
*his Attorney*

## UNITED STATES PATENT OFFICE

2,492,269

FLUID COOLED MEMBER FOR BLAST  
FURNACES AND THE LIKE

Robert T. Comer, Jr., Birmingham, Ala., assignor  
to Tennessee Coal, Iron and Railroad Com-  
pany, a corporation of Alabama

Application August 5, 1948, Serial No. 42,618

4 Claims. (Cl. 266—38)

1

This invention relates to improvements in water-cooled members for blast furnaces.

Due to the high temperatures generated in the hearth and bosh of blast furnaces, such as are used for smelting iron ore, and the erosive action of the molten iron and slag, it is necessary to provide means for cooling brickwork to prolong the life thereof. It has also been found necessary to cool the furnace openings through which the blast is introduced into the hearth, and through which the molten slag is drawn off between castings in order to withstand the intense physical, thermal and chemical action. Although many other metals have been tried, it is the general practice to use water-cooled copper or bronze castings for these purposes. This for the reason in spite of the relatively low melting point for copper or bronze, it holds up better than other metals because of its high coefficient conductivity. However, copper or bronze will not withstand long contact with the molten iron or slag and as a result, the castings are frequently burned, thus releasing water into the furnace causing delays in blast furnace operations while the burned castings are replaced. This replacement of burned water-cooled members constitutes a major source of delays in blast furnace operation and likewise some of the most serious interruptions due to chilled hearth and the like are brought on by failures of these water-cooled parts.

The problem of replacement is particularly acute with respect to so-called cinder notch "monkeys," i. e., the opening through which the slag is withdrawn from the furnace. Thus, the average life of bronze monkeys, in a blast furnace in accordance with a recent check, was 6.54, 6.93, and 5.98 days, respectively. The average delay for a burned monkey during this period was 28 minutes with a corresponding loss in tonnage and increase in cost.

It is accordingly an object of the present invention to provide water-cooled blast furnace castings having an increased life.

It is another object to reduce delays in blast furnace operation.

It is a further object to provide a blast furnace water-cooled monkey having a materially increased service life.

The foregoing objects will be apparent from the following specification which will particularly describe a blast furnace monkey in conjunction with the attached drawing, wherein:

Figure 1 is a longitudinal section of a blast furnace monkey embodying the teachings of my invention; and

Figure 2 is an end view thereof.

Referring more particularly to the drawing, the numeral 2 designates a hollow water-cooled

2

cast blast furnace monkey, preferably formed of cupreous metal, such as copper or bronze. The monkey provides a passage 4 in the brickwork wall 6 of the blast furnace (not shown) for the removal of the molten slag from the furnace. Cooling water is admitted to the monkey 2 through a suitable opening 8 and withdrawn through a similar opening 10. A baffle 12 may be provided intermediate the openings 8 and 10 to provide positive circulation of the cooling water through the internal cavity 14 in the cooling member.

Such members have the dual function of cooling the brickwork surrounding them and protecting the brickwork from the corrosive action of molten slag withdrawn therethrough. In order to better accomplish this latter function and, in accordance with the teachings of my invention, the inner exposed end portion 16 and the inside 18 through which the molten material passes are plated with a metal coating 20, the coating metal having a melting point in excess of the hearth temperatures in the furnace. With low silicon basic iron, the hearth temperatures will not exceed 2600° F. whereby a coating material having a melting point in excess of 2600° F. such as nickel which has a melting temperature of 2646° F. is quite satisfactory. However, for higher silicon irons, the hearth temperatures may run as high as 2750° F. so that for such material the coating metal should have a melting temperature in excess of 2750° F. I have found that chromium which has a melting point of 2990° F. is very satisfactory for all operations.

The coating metal, in order to achieve the objects of this invention and provide protection for the cupreous water-cooled member without lowering the cooling effect thereof, should have a thickness of the order called for by the following formula:

$$L_1 = \frac{K_1 \Delta T_1}{K_2 \Delta T_2} \cdot L_2$$

45 wherein

$L_1$ =thickness of chromium

$K_1$ =thermal conductivity of coating metal

$\Delta T_1$ =temperature drop in coating metal

$L_2$ =thickness of casting metal

50  $K_2$ =thermal conductivity of casting metal

$\Delta T_2$ =temperature drop in casting metal

While a coating having a slightly greater thickness may be used, it is essential that coating have 55 a thickness at least as great as that indicated by the foregoing formula.

Actual blast furnace operations have shown that cupreous monkeys coated with chromium of the foregoing thickness, have a service life in excess of 30 days as compared to the 5 to 6-day

average above noted. Similarly other water-cooled members used in blast furnaces, such as tuyères, tuyère coolers, bosh cooling plates, shell cooling plates, cinder coolers and the like, may have their life correspondingly increased without lowering the cooling efficiency thereof.

While I have shown and described one specific embodiment of my invention, it will be understood that this embodiment is merely for the purpose of illustration and description and that various other forms may be devised within the scope of my invention, as defined in the appended claims.

I claim:

1. A water-cooled member for blast furnaces comprising a hollow casting formed of cupreous metal, said casting having an external layer of metal having a melting point above 2600° F., said external layer having a minimum thickness determined by the formula

$$L_1 = \frac{K_1 \Delta T_1}{K_2 \Delta T_2} \cdot L_2$$

wherein

$L_1$ =thickness of the external coating  
 $K_1$ =thermal conductivity of coating metal  
 $\Delta T_1$ =temperature drop in coating metal  
 $L_2$ =wall thickness of casting metal  
 $K_2$ =thermal conductivity of casting metal  
 $\Delta T_2$ =temperature drop in casting metal.

2. A water-cooled member for blast furnaces comprising a hollow casting formed of cupreous metal, said casting having an external layer of metal having a melting point above 2750° F., said external layer having a minimum thickness determined by the formula

$$L_1 = \frac{K_1 \Delta T_1}{K_2 \Delta T_2} \cdot L_2$$

wherein

$L_1$ =thickness of the external coating  
 $K_1$ =thermal conductivity of coating metal  
 $\Delta T_1$ =temperature drop in coating metal  
 $L_2$ =wall thickness of casting metal  
 $K_2$ =thermal conductivity of casting metal  
 $\Delta T_2$ =temperature drop in casting metal.

3. A water-cooled monkey for blast furnaces comprising a hollow casting formed of cupreous metal, said casting having an external layer of chromium, said chromium layer having a minimum thickness determined by the formula

$$L_1 = \frac{K_1 \Delta T_1}{K_2 \Delta T_2} \cdot L_2$$

wherein

10  $L_1$ =thickness of the external coating  
 $K_1$ =thermal conductivity of coating metal  
 $\Delta T_1$ =temperature drop in coating metal  
 $L_2$ =wall thickness of casting metal  
 $K_2$ =thermal conductivity of casting metal  
 $\Delta T_2$ =temperature drop in casting metal.

15 4. A water-cooled monkey for blast furnaces comprising a hollow casting formed of cupreous metal, said casting having an external layer of chromium, said chromium layer having a thickness determined by the formula

$$L_1 = \frac{K_1 \Delta T_1}{K_2 \Delta T_2} \cdot L_2$$

wherein

25  $L_1$ =thickness of the external coating  
 $K_1$ =thermal conductivity of coating metal  
 $\Delta T_1$ =temperature drop in coating metal  
 $L_2$ =wall thickness of casting metal  
 $K_2$ =thermal conductivity of casting metal  
 $\Delta T_2$ =temperature drop in casting metal

30

ROBERT T. COMER, JR.

#### REFERENCES CITED

The following references are of record in the 35 file of this patent:

#### UNITED STATES PATENTS

| Number       | Name             | Date          |
|--------------|------------------|---------------|
| Re. 6,402    | Adams, Jr. ----- | Apr. 27, 1875 |
| 40 1,536,755 | Berg -----       | May 5, 1925   |
| 1,662,850    | Ebner -----      | Mar. 20, 1928 |
| 1,829,623    | Wright -----     | Oct. 27, 1931 |

#### FOREIGN PATENTS

| Number  | Country       | Date          |
|---------|---------------|---------------|
| 462,474 | Germany ----- | Mar. 14, 1926 |